

# UNITED STATES PATENT OFFICE.

CHARLES WILLIAM FISH, OF RAWCLIFFE, NEAR GOOLE, ENGLAND, ASSIGNOR TO THE AMBER SIZE & CHEMICAL COMPANY, LIMITED, OF LONDON, ENGLAND.

## MANUFACTURE OF PAPER AND THE LIKE.

1,229,924.

Specification of Letters Patent. Patented June 12, 1917.

No Drawing.

Application filed December 28, 1916. Serial No. 139,403.

To all whom it may concern:

Be it known that I, CHARLES WILLIAM FISH, a subject of the King of Great Britain and Ireland, and residing at Reedholme, 5 Rawcliffe, near Goole, in the county of York, England, have invented certain new and useful Improvements in the Manufacture of Paper and the like, of which the following is a specification.

10 This invention relates to a new or improved process of sizing pulp in the manufacture of paper and the like.

In the process ordinarily employed a size is added consisting of a resinate of soda. 15 This requires to be fixed, that is, decomposed into its components, resin and soda, so that the resin shall be freed from the soda in a finely divided state, one of the soluble aluminium salts, such as aluminium sulfate, 20 alum, or "alumino ferric cake" (sulfate of iron and alumina) being added for this purpose.

It has before been proposed to substitute the aluminium salts wholly by an acid bisulfate or by mixtures of aluminium sulfate and a bisulfate, but I have found by experiment that complete substitution does not give useful results, and that mixtures of aluminium salts with bisulfate of soda as 25 previously proposed are also objectionable, as difficulties arise from the two components being added to the pulp at the same time.

Now the object of the present invention is to substitute to a great extent for the 35 aluminium salts, niter cake or crude bisulfate of soda which is almost a waste product in the manufacture of nitric acid, hydrochloric acid and some other chemicals, so that the quantity of niter cake or crude 40 bisulfate may be considerably in excess of the aluminium salts.

After a large amount of experimenting on a manufacturing scale it has been found that the total substitution of alum by niter cake 45 was only practicable when making common grade papers. When the niter cake and the resinate of soda were alone employed, the troubles hereafter mentioned were largely encountered, whereas these troubles are 50 overcome or no longer exist in the improved process I now describe.

It is as follows: The size is added to the pulp in the beating engine thoroughly mixed, then a small percentage of alum, say

half per cent. to one per cent. of the pulp, 55 is added, varying in amount according to the hardness of the water used, and also to the degrees of sizing required in the paper and the class of material employed. After this has become thoroughly distributed in 60 the pulp the niter cake is added, the weight of niter cake used being usually about the same for each class of material as the amount of alum ordinarily employed, less perhaps the small amount already added. 65 The quantity of alum, however, required varies greatly with different classes of paper, but this is well known to the trade and therefore the amount of niter cake can be very easily determined.

70 I find practically that one part of niter cake containing 75 per cent. bisulfate of soda replaces one part of alum.

One thing, however, is essential: the niter cake must be added last. If this is not done 75 the mineral colors usually added in the beating engine are not thoroughly fixed and the press bowls are rendered very dirty and sticky by the resin accumulating on them. This again causes the web of paper to break 80 down and this upsets the running of the machine: the pores of the wires also become filled up, causing "imperfect paper." The rolls of the machine also become coated with particles of resin and cause the fibers 85 or particles of pulp to stick to them, and in the case of M. G. single cylinder machines, commonly known as Yankee, the finish is seriously interfered with owing to 90 resin being conveyed from the paper on to the cylinder producing unglazed patches and blotches or specks of resin on the paper.

95 Not only is the paper harder when sized by my process but the coloring matter, especially artificial organic colors and dye stuffs whether basic acid or salt and even the mineral colors, such as ocher and the like, and other inorganic pigments such as chrome yellow, Prussian blue paste and the like, are well fixed in and on the fiber, thus insuring good shades being obtained.

100 By my process also very considerable economy of cost is obtained over any other sizing process I am acquainted with.

As illustrations of my process I give the 105 following cases of actual manufacture which have been very successful.

12 cwt. of strong unbleached air-dried

sulfite pulp is filled into the beater and at the same time 7 lbs. of alum and 40 lbs. of size, containing 30 per cent. to 35 per cent. of resinate of soda, are added. After these have become thoroughly mixed with the pulp 5 20 lbs. of niter cake are added, preferably broken up into small lumps, and the requisite amount of water added. The beater in a short time thoroughly mixes these materials. In practice about 92 per cent. of water is added to 8 per cent. of air-dried fiber.

Again, in the case of M. G. envelops about D. C. 30 to 40 lbs., 7 lbs. of alumino ferric is first added when filling into the beater 15 with the usual quantity of water 11 cwts. of a mixture consisting of 65 per cent. of mechanical wood pulp and 35 per cent. strong unbleached sulfite pulp reckoned dry, then 100 lbs. of size 32 per cent. strength is 20 added and after that 40 lbs. of niter cake (containing 87 per cent. bisulfate of soda, 9 per cent. sulfate of soda and 4 per cent. water).

These two illustrations will show the general working of my invention but in every different variety of pulp and for nearly every different use the quantities differ to some extent.

The main features of my invention are: 25 (1) the addition of a very small percentage of alum, and (2) the thorough mixture and

solution in the furnish before the niter cake is added.

I find that to secure successful results it is necessary to add the niter cake after the 35 size and alumina salts have been introduced into the pulp.

Having now particularly described and ascertained the nature of my said invention and in what manner the same is to be performed, I declare that what I claim is:—

1. In the process of sizing pulp for the manufacture of paper or the like using niter cake and alumina salts for fixing the size, the addition of the niter cake separate 45 from the alumina salts and only after the size and the alumina salts have been incorporated in the pulp, substantially as described.

2. In the process of sizing pulp for the 50 manufacture of paper and the like, thoroughly mixing the requisite quantity of resin size with the pulp and adding a small quantity of a soluble alumina salt, say half per cent. to one per cent. of the stuff in the beater, and when these are thoroughly mixed adding bisulfate of soda or niter cake, 55 substantially as described.

In testimony whereof, I have affixed my signature.

CHARLES WILLIAM FISH.